

1

3,384,575

PETROLEUM REFINING WITH ORGANIC  
ACID ANHYDRIDES  
Charles O. Hoover, 502 Princess Drive,  
Corpus Christi, Tex. 78410  
No Drawing. Filed May 24, 1965, Ser. No. 458,461  
4 Claims. (Cl. 208—285)

## ABSTRACT OF THE DISCLOSURE

A process for treating petroleum stocks to improve their storage stability by successive admixture with the stock of first, an organic acid anhydride, and second, sodium methylate in an amount sufficient to neutralize the admixture.

This invention relates to the refining of petroleum, and more particularly to the chemical refining of petroleum including both crude petroleum and the fractions produced therefrom in the course of processing the crude petroleum.

Most crude petroleums include sulfur compounds, phenolic and nitrogenous bodies, acids and the like which impart to the various fractions produced in the processing of the crude petroleum undesirable physical and chemical characteristics. These undesirable characteristics include bad odor, sourness to the conventional "doctor" test, poor color stability in storage, formation of gummy precipitates in storage which, in the case of household fuel oils, are particularly deleterious. In the case of gasoline fractions, these undesirable constituents also frequently reduce the clear octane values of the fractions, as well as the lead susceptibility thereof.

Processing of the crude oil under the temperature and pressure conditions normally applied, frequently intensifies the undesirable characteristics noted. In catalytic cracking of petroleum fractions there is produced refractory recycle stock which is withdrawn from the system and includes a large proportion which falls in the household fuel or burning oil range. This is commonly referred to as "light cycle oil" or "No. 2 fuel oil." This material is found to be unstable in storage, losing color rapidly and developing gummy precipitates and possessing highly undesirable odors, all of which make the product undesirable and often a source of mechanical difficulty in use.

Various processes are presently employed in an effort to render these burning oil stocks satisfactory for their intended use. Among the more extensively used processes is hydrogenation which necessarily involves expensive equipment and high operating costs. Another process used is the treatment of the oil with concentrated caustic soda solution followed by subjecting the alkali treated oil to the action of electrical precipitators in order to remove, to the greatest extent possible, traces of the alkali reaction products which would otherwise remain suspended in the oil. This process, too, requires expensive equipment and relatively high treating costs.

In my U.S. Patent No. 2,889,195, I have disclosed a comparatively simple chemical treatment by which the various petroleum distillates which possess the aforementioned undesirable characteristics may be rendered entirely free of these characteristics.

In the patented process, I employ as the chemical reagents, an organic acid anhydride, preferably acetic anhydride, and concentrated aqueous alkali hydroxide solution, preferably sodium hydroxide in a concentration of at least 25% by weight of the alkali solution.

I have now discovered that by substituting sodium methylate for the alkali hydroxide as used in the patented process, I not only obtain the desired results, so far as im-

2

proving the quality of the oil is concerned, but I am able to very markedly reduce the quantity of chemicals required and the cost thereof. By employing sodium methylate, generally in a methanol solution, I have found that the quantity of organic acid anhydride, as required in the earlier process, may be reduced by as much as 90%, or even more, and the quantity of sodium methylate required will be in the range of from about 5% to 15% of the amount of caustic alkali previously required.

As in the case of the patented process, the process of the present invention may be applied to the various petroleum distillates at appropriate stages following their production in conventional refining operations, or may be applied to the crude petroleum itself prior to subjecting it to the usual processing operations. In the case of the catalytically cracked cycle stocks, the process will usually be applied to the cycle stock in order to obviate the undesirable properties imparted to this material by the catalytic treatment.

The process in accordance with this invention comprises the liquid phase chemical treatment of petroleum by two reagents applied to the oil in succession under controlled conditions.

In accordance with the preferred embodiment of this invention, the first treatment stage comprises, thoroughly admixing with the oil a small proportion of acetic anhydride and thereafter, without intermediate settling or other processing, the second stage comprises vigorously admixing with the oil containing the acetic anhydride, a small quantity of sodium methylate (sodium methoxide), preferably in a methanol solution. Because of the relatively minute amounts of chemicals required to complete the reactions involved, the reaction products usually will be so small in quantity that they may be permitted to remain in the treated oil without any deleterious effect.

As indicated previously, it is one of the unexpected results of the substitution of sodium methylate for aqueous alkali solutions of the patented method, that the total quantity of reagents, including the acid anhydride, is reduced to such a small quantity, both relatively and in absolute terms, that no separating step for reaction products will ordinarily be required, and it is further found that the reaction products, whatever their character, when left in the oil, do not, as noted previously, have any adverse effect on the stability of the oil.

It is found that treatment of the oil by the process described, removes undesirable odors; renders the oil completely stable to the standard stability test (which comprises subjecting a sample of the oil in an open container to a temperature of 212° F. for 24 hours), the resulting stability obviating color loss or formation of precipitates. In many instances, the oil will be rendered sweet to the conventional "doctor" test.

In the case of gasoline distillates, the treatment frequently results in improvement in the clear octane values of such stocks, as well as improving the lead susceptibility thereof.

The mechanisms of the reactions which occur in the treating process of the present invention is not fully understood, but it is thought that some type of acylation reaction occurs between the acetic anhydride (or other anhydride employed) and the mercaptans and other types of sulfur bodies in the oil, and with the nitrogenous bodies and phenolic or other hydroxy or carboxylic compounds which may be present. It will be understood, therefore, that this invention should not be considered as dependent upon any specific reaction mechanism or theory, but is to be based upon the procedure employing certain specified reagents as herein set forth.

As indicated previously, acetic anhydride is my preferred reagent for the first stage treatment, and sodium

methylate, preferably in the form of a 25% solution in methanol, for the second stage treatment.

Acetic anhydride is preferred because of its readily commercial availability and comparatively low cost, although other acid anhydrides, both aliphatic and aromatic may be used, but are generally more expensive and not as efficient, in some instances, as the preferred acetic anhydride. Other anhydrides include propionic, butyric and hexanoic anhydrides in the aliphatic category, and phthalic and benzoic anhydrides in the aromatic category. The latter, being normally solids, must first be dissolved in a suitable solvent, such as benzol, which will be fully miscible with the oil being treated. Mixtures of the anhydrides can also be used.

The entire procedure in accordance with this invention is a liquid phase treating process which is normally conducted at atmospheric temperatures and pressures, although where light gasoline distillates are treated, the operation may be conducted in a closed system under sufficient pressure to prevent vaporization and loss of light fractions.

The anhydride, preferably acetic anhydride, is added to the oil in proportions varying generally with the character and source of the oil being treated. In general, only a very small amount of acetic anhydride is necessary, this amount being in the range from about 0.001% by volume to about 0.005% by volume of the oil being treated. In the case of light cycle oil from catalytic cracking, generally from about 0.002 to 0.005% by volume of acetic anhydride will be found to be most generally applicable. In the case of crude oil or other stocks having relatively large proportions of impurities, these quantities may be increased to 5 to 10 times the amounts heretofore stated.

The amount of the acetic anhydride and the time of contact with the oil must be such that after subsequent treatment of the mixture of the acetic anhydride and oil with the sodium methylate solution, a sample of the treated oil heated in an oven at 212° F. for 24 hours shows an improved color as compared to an untreated sample of the same oil heated at the same temperature for the same time.

The sodium methylate solution is added to the admixture of the oil with the acetic anhydride following the addition of the latter. The time interval between the additions to the oil of the first and second reagents is variable, it being only important that the acetic anhydride be thoroughly mixed with the oil before the sodium methylate solution is admixed therewith. While ordinarily the sodium methylate will be added immediately after completion of the mixing of the acetic anhydride with the oil, the treatment may be successfully effected even though the sodium methylate is added hours or days after the addition of the acetic anhydride to the oil.

It appears that whatever may be the reactions which occur between the acetic anhydride and the constituents of the oil, these reactions occur substantially instantaneously so that it is only necessary to employ sufficient mixing to assure that the acetic anhydride has been thoroughly distributed through the oil before the sodium methylate solution is applied. It is important to note, therefore, that the reagents should be added separately and successively, the sodium methylate solution following the anhydride addition, but that the time interval between the additions of the reagents is not particularly important.

The quantities of sodium methylate added is quite small and is added in amounts generally sufficient to neutralize any excess anhydride or acidic reaction products which may be formed, as calculated from the neutralization number of the oil as determined by the standard ASTM Test D-664-58. In general, the quantities of sodium methylate required for most oil stocks will range from about 0.001% to about 0.05% by volume of the oil. For burning oils the quantities required

will be in the range from about 0.005% to about 0.03% by volume of the oil.

As sodium methylate is a highly hygroscopic powder which will be decomposed violently by water, it is ordinarily employed in a methanol solution which may, of course, be varied in its concentration of sodium methylate. As noted previously, a 25% solution of the reagent in methanol is found generally preferable, but this concentration may be varied if preferred. Since, as noted, the quantities of the reagents, particularly the sodium methylate solution, is extremely small, there is usually no necessity for any settling or separation of products of the reaction. Hence, the process may be termed a "once-through" process.

The time of treatment of the oil with the acetic anhydride should be sufficiently long to assure adequate mixing and will vary somewhat, depending upon the volumes treated. Usually 15 seconds to 5 minutes will be found adequate, but longer times may be employed. The subsequent treatment with the sodium methylate solution is likewise dependent mainly upon the degree of agitation to be applied and as much time as may be found necessary to assure complete and thorough mixing of the sodium methylate solution with the oil-anhydride mixture will be required. This time may be of the order of a few seconds to several minutes.

By way of comparison with the chemical requirements of the treating process disclosed in my aforesaid U.S. Patent No. 2,889,195, the following results were obtained in comparing the treatments, on a commercial scale on the order of 5,000 barrels per day, of a light cycle oil from catalytically cracked stock. Where the patented process required 0.03% by volume of the oil of acetic anhydride, the present process required 0.0025% of acetic anhydride, and where the patented method required 0.10% by volume of a 25% aqueous solution of sodium hydroxide continuously circulated at a rate of about 5% by volume of the oil, the present method required the admixture with the oil-anhydride solution of 0.005% by volume of a 25% methanol solution of sodium methylate. In the case of both reagents, it will be seen that the volumetric requirements were reduced by 95% or more, and, of course, in the present process, no recirculation of the sodium methylate or separation of reaction products were required.

Following are some additional examples of treating various heating oils with the present method:

#### EXAMPLE I

A heating oil with an acid value of 0.03 mg. KOH/g., and having an initial union color of 1½+ when subjected to an accelerated storage stability test (vented storage at 212° F. for 24 hours) deteriorated to an 8+ color. This oil was treated by dissolving in the oil 0.002% by volume acetic anhydride and then by vigorous agitating the oil with 0.011% by volume of sodium methylate (25% solution in methanol) a very small amount of insoluble reaction product was formed and separated from the oil. The separated oil had a storage stability color of 2-.

#### EXAMPLE II

Another heating oil with an acid value of 0.01 mg. KOH/g. and an initial union color of 2- gave an accelerated storage stability color of 8+. This oil was treated with 0.0025% by volume of acetic anhydride followed by 0.03% by volume of sodium methylate (25% solution in methanol) and after separation from the minute amounts of insoluble reaction products which developed, produced an oil having storage stability color of 2 on the union colorimeter scale.

#### EXAMPLE III

Still another heating oil having an acid value of 0.02 mg. KOH/g., an initial union color of 1½+ and a union color of 5, after 24 hours at 212° F. was treated with

0.0027% by volume of acetic anhydride followed by 0.0173% by volume of sodium methylate (25% solution in methanol) and without separation of any precipitate, produced a treated oil which maintained a 1½+ union color on the storage stability test.

From the foregoing, it will be seen that the present invention provides an exceptionally effective, simple, low cost process for the treatment of petroleum oils by which outstanding improvement in the physical and chemical properties thereof is effected. Distillate products such as the gasoline fractions and burning oil fractions, when treated by the method in accordance with this invention, become finished stocks, requiring no further processing before use.

What I claim and desire to secure by Letters Patent is as follows:

1. The method of refining petroleum oil, comprising, admixing with a petroleum oil stock in the liquid phase an organic acid anhydride selected from the group consisting of acetic, propionic, butyric, hexanoic, phthalic and benzoic anhydrides in an amount ranging from about 0.001% to about 0.005% by volume of the oil stock, and thereafter agitating the admixture with sodium methylate in an amount sufficient to neutralize said admixture.

2. The method of refining petroleum according to claim 1, wherein the quantity of sodium methylate added is in the range from about 0.001% to about 0.05% by volume of the oil stock.

3. The method according to claim 1, wherein said petroleum oil stock is the light cycle stock, commonly designated as "No. 2 fuel oil," obtained from the catalytic cracking of petroleum.

4. The method according to claim 1, wherein said organic acid anhydride is acetic anhydride.

10

#### References Cited

##### UNITED STATES PATENTS

|           |         |                |       |         |
|-----------|---------|----------------|-------|---------|
| 2,068,850 | 1/1937  | Ellis          | ----- | 208—282 |
| 2,769,766 | 11/1956 | Folkins et al. | ----- | 208—282 |
| 2,889,195 | 6/1959  | Hoover         | ----- | 208—285 |

##### FOREIGN PATENTS

|         |         |          |
|---------|---------|----------|
| 401,353 | 12/1938 | Germany. |
|---------|---------|----------|

DELBERT E. GANTZ, *Primary Examiner.*

GEORGE J. CRASANAKIS, *Assistant Examiner.*

15

20